

## UNITED STATES PATENT OFFICE

2,121,684

## ARTIFICIAL LEATHER

Merlin Martin Brubaker, Wilmington, Del., and  
Leo Phillip Hubbuch, Springfield, Pa., assign-  
ors to E. I. du Pont de Nemours & Company,  
Wilmington, Del., a corporation of Delaware

No Drawing. Application June 15, 1936,  
Serial No. 85,416

2 Claims. (Cl. 91—68)

This invention relates to artificial leather products and more particularly to fabrics coated with cellulose derivative compositions.

This application is a continuation in part of 5 our application Serial Number 691,094, filed September 26, 1933.

This invention has as an object the preparation of new and useful coated fabrics. A further object is the manufacture of artificial leather products comprising cellulose nitrate coated fabrics 10 possessing exceptional toughness, abrasion resistance, and durability. A still further object is the production of coated fabrics of this kind in which the cellulose derivative coating possesses an unusually high exudation temperature. Other objects will appear hereinafter.

These objects are accomplished by the following invention wherein suitable fabrics are coated with cellulose derivative compositions softened 20 by synthetic oils prepared by the chemical combination of a dibasic organic acid, a dihydric alcohol, and definite proportions of a fatty acid glyceride of the coconut oil type, i. e., a fatty acid glyceride having an iodine number of less than 35 and a saponification number of 200 to 25 300. It has been discovered that glycerides of the coconut oil type may be modified so as to render them of great utility in cellulose derivative compositions applied over flexible fabrics.

In order that softening agents for cellulose derivative compositions shall retain their initial properties on aging it has been found that the softening agent should be almost saturated to 35 prevent its oxidation and the detrimental effect of this oxidation on the remainder of the cellulose derivative composition. Hereinafter the term "saturated" when used with reference to glycerides of the coconut oil type includes only those glycerides with an iodine number below 40 35. An iodine number of about 85 corresponds roughly to a glyceride from a long chain fatty acid containing one double bond. The saponification values of a few pure glycerides may be listed, thus, tristearin 189, tripalmitin 208, tri-45 laurin 263, tricaprin 304. The saponification value is the number of milligrams of potassium hydroxide required to saponify one gram of the oil, fat or wax.

The examples given below in which the parts 50 are by weight illustrate the more specific details of the invention. The first three of these examples describe the preparation of the softener constituent of the cellulose derivative coat.

## Example I

| Constituent:                      | Parts |
|-----------------------------------|-------|
| Diethylene glycol (mol. wt. 106)  | 15.4  |
| Coconut oil (mol. wt. 662)        | 61.3  |
| Glycerol (mol. wt. 92)            | 0.9   |
| Phthalic anhydride (mol. wt. 148) | 22.4  |

The diethylene glycol, coconut oil, and glycerol are heated together in a closed kettle, fitted with a reflux condenser and stirrer for one hour at 250° C., or until a test spot of the mixture on cooling does not become cloudy. This alcoholysis step is facilitated by very rapid stirring. At the completion of the alcoholysis the charge is cooled slightly and the phthalic anhydride is added. Steam is blown through the condenser, and CO<sub>2</sub> is blown through the charge which is stirred rapidly and heated for six hours at 225° C. At this point, the acid number of the product is approximately 5.0. The charge is then cooled. The resulting product is a light brown oil of viscosity around nine poises. In place of the oil, it is understood that the requisite amounts of oil acids and glycerol may be used and the initial alcoholysis step avoided. However, the alcoholysis method is preferred inasmuch as it gives a better product.

In place of diethylene glycol, some other dihydric alcohol such as ethylene glycol may be used. The following example illustrates this use:

## Example II

| Constituent:                      | Parts |
|-----------------------------------|-------|
| Ethylene glycol (mol. wt. 62)     | 10.30 |
| Coconut oil (mol. wt. 662)        | 67.30 |
| Glycerol (mol. wt. 92)            | 0.10  |
| Phthalic anhydride (mol. wt. 148) | 22.30 |

The ethylene glycol, coconut oil, and glycerol are heated together in a closed kettle fitted with a reflux condenser and stirred for 1½ hours at 200° C. until some alcoholysis has occurred. This alcoholysis step is facilitated by very rapid stirring. The charge is then cooled and the phthalic anhydride added. Steam is blown through the condenser and CO<sub>2</sub> is blown through the charge which is stirred rapidly and heated for four hours at 225° C. At this point, the acid number of the product is approximately 5.0. The charge is then cooled. The resulting product is a light brown oil of a viscosity around nine poises.

Other proportions of the polybasic acid—dihydric alcohol constituent and the saturated glyceride of the coconut oil type may be used as the following example will illustrate:

## Example III

| Constituent:                      | Parts |
|-----------------------------------|-------|
| Diethylene glycol (mol. wt. 106)  | 19.18 |
| Coconut oil (mol. wt. 662)        | 43.70 |
| Coconut oil acids (mol. wt. 208)  | 22.70 |
| Phthalic anhydride (mol. wt. 148) | 14.42 |

The diethylene glycol, coconut oil, coconut oil acids, and phthalic anhydride are heated together in a closed kettle fitted with a stirrer and a steam reflux condenser for eight hours at 225° C. During the heating the charge is stirred moderately and blown with CO<sub>2</sub>. After eight

hours' heating, the charge shows an acid number of around 2.0. The product, when cooled, is a light red oil of a viscosity around five poises. In the above example both the coconut oil and 5 the coconut oil acids are used. This is found essential in order to obtain the desired composition.

The following two examples illustrate compositions which contain the foregoing softeners and 10 which are applied to the flexible fabric in the manufacture of my improved artificial leather products:

*Example IV*

|                               | Parts |
|-------------------------------|-------|
| 15 Softener of Example III    | 18.4  |
| Extracted pyro nitrocellulose | 11.8  |
| Lithopone pigment             | 13.6  |
| Ethyl acetate                 | 22.4  |
| Ethyl alcohol                 | 33.8  |

20 This composition, when spread on cloth and suitably dried, gives an artificial leather which is superior to that with castor oil or coconut oil as the softener.

*Example V*

|                               | Parts |
|-------------------------------|-------|
| 25 Softener of Example I      | 20.8  |
| Extracted pyro nitrocellulose | 11.3  |
| Lithopone pigment             | 14.4  |
| Ethyl acetate                 | 21.4  |
| 30 Ethyl alcohol              | 32.1  |

The softeners should not for the best results contain substantially more than the amount of coconut oil glyceride used in the above examples. 35 As the proportion of the oil glyceride gets greater than about 70% the advantageous properties, particularly with respect to toughening action and freedom from exudation, become less pronounced. The minimum amount of the coconut 40 oil glyceride is about 40% and the optimum results are obtained from 60 to 65%.

In the foregoing description the invention has been outlined in relation to coconut oil, ethylene glycol, diethylene glycol, and phthalic anhydride. 45 Other glycerides of the coconut oil type, other dihydric alcohols and other dibasic acids may, however, be used in varying proportions. Changes in the ratio of glyceride to dihydric alcohol-dibasic acid complex are of course necessary depending 50 on the glyceride, the dihydric alcohol, and the dibasic acid. For coconut oil other saturated glycerides of the coconut oil type such as those mentioned above may be substituted. In place 55 of diethylene glycol or ethylene glycol, other dihydric alcohols such as triethylene glycol, butylene glycol, dipropylene glycol, octadecanediol, monobenzylin, propylene glycol, monoethylin, monomethylin, may be used. Other dibasic acids or their equivalent derivatives such as the anhydride may be used, such as succinic, adipic, diphenic, camphoric, tartaric, malic, pimelic, sebacic, suberic, azelaic, etc., acids.

The methods of preparing the softeners used in our new products may vary considerably. The 65 preferred method is to heat the saturated glyceride with the dihydric alcohol so as to obtain alcoholysis, and to prevent as much as possible the formation of the dibasic acid-dihydric alcohol complex when the dibasic acid is later added. 70 It is, however, possible to prepare similar products by heating all of the constituents together simultaneously or, in certain cases, by forming the dihydric alcohol-dibasic acid complex first and heating this with the saturated glyceride. 75 The acids of the saturated glyceride may be

heated with the requisite amount of glycerol in the presence of one or more of the other constituents, the remaining ingredients being added at a later stage of the heating to produce suitable softeners. The resin may also be prepared 5 in the presence of an inert solvent as described in the co-pending application of M. M. Brubaker, Serial Number 421,585, filed January 17, 1930. Experience, however, has shown that the alcoholysis method for the preparation of non-blooming, 10 stable softeners is by far the best.

The total effect of a softener for artificial leather compositions is a resultant of two distinct effects, i. e., viscosity and solvent action. Increasing the viscosity of the softener, within 15 certain limits, increases the strength and binding power of the coating composition, increases its exudation temperature and decreases its pliability. Increasing the solvent action of the softener, within certain limits, decreases the strength 20 of the coating composition, increases its exudation temperature and increases its pliability. By proper adjustment of these two effects it is possible to arrive at a softener which, with cellulose derivatives, gives a film of good toughness, and a 25 high exudation temperature at a pliability suitable for a coating for a flexible backing. However, in order to secure the proper pliability of the film it is necessary to change the ratio of the softener to the cellulose derivative depending 30 upon the viscosity and solvent action of the softener. In making these new castor oil substitutes the non-solvent glyceride such as coconut oil is heated with a dihydric alcohol such as diethylene glycol and ester interchange occurs 35 with the partial formation of a dihydric alcohol ester which has some solvent action.

By adding phthalic anhydride and esterifying, the viscosity of the softening agent is increased due to the formation of some dibasic 40 acid-dihydric alcohol complex. If the viscosity of the softener is increased too much (roughly, greater than 250 poises) by the formation of a large proportion of the dibasic acid-polyhydric alcohol complex, e. g. that obtained from more 45 than 40% phthalic anhydride, it is not possible to obtain a tough, abrasion resistant film of the proper pliability with a cellulose derivative even by increasing the ratio of softening agent to the cellulose derivative. In other words without the combined dibasic acid-dihydric alcohol reaction products, the glycerides fail to give binding power to the other ingredients of the artificial leather coating composition, or else bloom from 50 the film; with too great a proportion of the combined dibasic acid-dihydric alcohol reaction products, the resulting softeners cause brittleness of 55 the coating composition.

Glycerides whose saponification values are 60 higher than 300, even after modification by the herein described process show too much solvent action on the cellulose derivative composition thereby reducing its toughness. Glycerides whose saponification values are lower than 200 are, even 65 after modification, too waxy and bloom from the film. A number of saturated glycerides of the coconut oil type are available for use. The large majority, however, are either not compatible with the cellulose derivative or else, due to their solid nature at room temperature tend to bloom from 70 a film containing them, i. e. tend to form a white, greasy, film on the surface of the cellulose derivative compositions. By modifying these saturated glycerides in the manner of this invention 75 oils ranging in viscosity from about 1 poise to 75

about 250 poises are obtained. These are readily compatible with cellulose nitrate and ethyl cellulose and show no tendency to bloom. Their compatibility with cellulose acetate is not particularly advantageous. While the advantage of non-blooming is pronounced, it is not the paramount one of the invention. In the judgment of the initial quality of artificial leather, two factors are important. The first is that the softening 5 component of the cellulose derivative and particularly cellulose nitrate coating composition must not exude or come out on the surface of the film in the form of oil drops at too low a temperature. In general, exudation much below 60° C. 10 indicates an incompatible film. A softener in a cellulose nitrate composition which does not exude until the temperature is at least 60° is a fair softener. One which exudes only above 80° is a good softener, and an excellent softener exudes 15 only at above 100°. The optimum is, of course, no exudation at any reasonable temperature. The second factor of importance, in the judgment of the initial quality of artificial leather, is the ability of the coated fabric to withstand scrubbing. 20 By the term "scrubbing" is meant rubbing two coated faces of the artificial leather together in a suitable manner until the coating is broken. The number of "scrubs" is considered a measure of the toughness of the coating. 25 The superiority of products described herein is illustrated by the following table which gives actual results on artificial leathers containing different softeners: 30

lar weight than stearic acid are excluded from the scope of the present invention because of this objectionable feature. Glycerides lower than tricaprin are also excluded since products of bad odor, high volatility and extreme solvent action are formed from such glycerides. 5

The superiority of our improved coated fabrics over similar products now in use for artificial leather is best shown by the following comparison: 10

| Composition                                                      | **Softener N/C ratio | Initial number of scrubs | Exudation temp. °C. | *Percent deterioration |
|------------------------------------------------------------------|----------------------|--------------------------|---------------------|------------------------|
| Example IV                                                       | 55:45                | 120                      | 96                  | +50                    |
| Same as Example IV with castor oil in place of the new softener  | 70:30                | 145                      | 63                  | +90                    |
| Same as Example IV with coconut oil in place of the new softener | 70:30                | 100                      | 77                  | +71                    |

\*The percent deterioration represents the decrease in scrub after four weeks' aging at 65° C.

\*\*Ratio of softener to nitrocellulose required to give a coating of medium pliability when 30% of pigment is used.

From this it is seen that after four weeks' aging at 65° C. the composition of Example IV would still scrub approximately 60 times before breaking, whereas the castor oil composition would scrub only approximately 15 times, and the coconut oil composition only approximately 29 times. In addition, both the castor oil and the coconut oil compositions exuded at tempera- 30

| 35                 | Softener ingredients | Percent | ***Softener | Initial | Exudation | Bloom |
|--------------------|----------------------|---------|-------------|---------|-----------|-------|
|                    |                      |         | N/C ratio   |         |           |       |
| Coconut oil        | 100.00               | 70:30   | 100         | 77      | Definite. |       |
| Coconut oil        | 43.70                |         |             |         |           | 40    |
| Coconut oil acids  | 22.70                |         |             |         |           |       |
| Dimethylene glycol | 10.18                | 55:45   | 120         | 96      | None.     |       |
| Phthalic anhydride | 14.42                |         |             |         |           |       |
| *Coconut oil       | 61.30                |         |             |         |           |       |
| Diethylene glycol  | 15.40                |         |             |         |           |       |
| Glycerol           | .90                  | 60:40   | 180         | 99      | None.     |       |
| Phthalic anhydride | 22.40                |         |             |         |           |       |
| *Coconut oil       | 43.30                |         |             |         |           | 45    |
| Diethylene glycol  | 10.44                |         |             |         |           |       |
| Glycerol           | 9.26                 | 75:25   | 80          | 170     | None.     |       |
| Phthalic anhydride | 37.00                |         |             |         |           |       |
| **Coconut oil      | 34.32                |         |             |         |           |       |
| Diethylene glycol  | 8.28                 |         |             |         |           |       |
| Glycerol           | 13.40                | 85:15   | 0           | 170     | None.     |       |
| Phthalic anhydride | 44.00                |         |             |         |           |       |
| **Coconut oil      | 31.90                |         |             |         |           | 50    |
| Diethylene glycol  | 22.10                | 85:15   | 0           | 170     | None.     |       |
| Glycerol           | 4.40                 |         |             |         |           |       |
| Phthalic anhydride | 41.60                |         |             |         |           |       |
| Stearin            | 100.00               | 70:30   | 0           | Low     | Bad.      |       |
| Castor oil         | 100.00               | 70:30   | 145         | 65      | None.     |       |

55 \* Improved castor oil substitutes of the present invention.

\*\* Balsams, i. e., resinous products.

\*\*\* Ratio of softener to nitrocellulose required to give a coating of medium pliability when 30 percent of pigment is used.

Typical balsams of the modified polyhydric alcohol-polybasic acid resin type outside of the 60 range of the products of this invention are unsuitable as castor oil substitutes in artificial leather compositions because of the brittleness they impart to the film. By the term "brittleness" as used herein is meant that characteristic of the 65 film coating composition which causes it to crack under a sudden sharp bend or other stress even though the film feels pliable and yields easily under a slow bending.

Experience with products of the present kind 70 and comparison with materials which might be deemed analogous have shown that stearin or its modifications prepared by the process of the present invention always blooms badly from the coating composition after the same has dried.

75 Stearin and glycerides of acids of higher molecu-

tures much lower than the composition of Example IV.

It may be mentioned that the softeners of the 60 present invention are hydrolyzed by boiling with caustic alkalies to yield salts of fatty acids similar to those in coconut oil, glycerol, a dihydric alcohol, and a salt of an organic dibasic acid. The organic dibasic acid is present to the extent of less than 40% of the total weight of products obtained by the hydrolysis and subsequent acidification.

It will be seen from the foregoing description 70 that we have developed an improved cellulose derivative coating peculiarly adapted to the manufacture of artificial leather products by reason of its extreme toughness, at practical pliabilities for artificial leather products, coupled with good 75

stability on aging and high exudation temperature.

As many apparently widely different embodiments of this invention may be made without departing from the spirit and scope thereof, it is to be understood that we do not limit ourselves to the specific embodiments thereof except as defined in the appended claims.

We claim:

- 10 1. An artificial leather product which comprises a flexible fabric sheet provided with a tough, pliable coating of cellulose nitrate composition containing a softener consisting of a syn-

thetic oil which comprises in chemical combination phthalic acid, a dihydric alcohol, and 40 to 70% by weight of the glyceride of coconut oil, said coating having an exudation temperature greater than 80° C. and having a high resistance to breaking upon rubbing coated faces of the artificial leather product together.

2. The artificial leather product set forth in claim 1 in which the coconut oil glyceride is present in amount from about 60 to 65% by weight. 10

MERLIN MARTIN BRUBAKER.  
LEO PHILLIP HUBBUCH.